

## UNITED STATES PATENT OFFICE.

LOUIS AEBY, OF EAST CHICAGO, INDIANA, ASSIGNOR TO CHICAGO FLEXIBLE SHAFT COMPANY, OF CHICAGO, ILLINOIS, A CORPORATION OF ILLINOIS.

## CARBURIZING MATERIAL AND PROCESS OF MAKING SAME.

No Drawing.

Application filed February 11, 1921. Serial No. 444,145.

*To all whom it may concern:*

Be it known that I, LOUIS AEBY, a citizen of the United States, having residence in East Chicago, in the county of Lake 5 and the State of Indiana, have invented certain new and useful Improvements in Carburizing Materials and Processes of Making Same, of which the following is a specification, reference being had to the accompanying drawings, forming a part thereof.

The purpose of this invention is to provide an improved material for case carburizing and a process for making the same. 15 It consists as to the material in the combination of the substances intermixed and united as described, and as to the process in the succession of steps as particularly set forth, all as indicated in the claims.

20 In the carrying out of this invention I reduce charcoal to a dust condition by any suitable pulverizing apparatus; and at any convenient stage in the process of such reduction, preferably before it is entirely 25 complete,—that is, before the charcoal is all reduced to a condition of dust, I intermix with the charcoal a suitable proportion of any convenient non-liquid energizer, as lime, soda-ash, sodium carbonate or 30 barium carbonate, such energizers becoming reduced to a dust condition in the continuing process of mixing them with the charcoal while completing the process of reducing that material to dust. During the 35 latter part of this process after the energizer is added to the charcoal, there is added a limited quantity of coal tar, or other binder only enough when thoroughly intermixed during the closing stage of the process of mixing the other elements to render the whole mass cohesive and moldable; and when the coal tar is thus thoroughly intermixed, so as to render the entire mass cohesive, it is molded into briquettes and 45 baked to dryness, primarily for the purpose of shrinking, at a temperature not suffi-

cient to fuse the energizer. These briquettes may in special cases where extended flat surfaces are to be case-hardened, be employed in their integral form; but in 50 general, these briquettes are crushed by any convenient crushing and fragmentizing apparatus and the crushed material is screened to sort it into different sizes and separate the dust which is too fine for desirable 55 use in case carburizing. This dust is returned to the mixing apparatus and mixed with the pulverized charcoal in the subsequent batches. In the continuous process of manufacture, the quantity of dust 60 returned from the crushed briquette, having of course a small quantity of coal tar, is substantially uniform so that variation in output from this cause is negligible.

I claim:

1. The process of making carburizing material which consists in the following steps; (1) mechanically reducing charcoal to a condition of dust; (2) at a stage in the process of such reduction to dust mechanically thoroughly intermixing with the charcoal and energizer adapted to be itself reduced to a condition of dust in the process of mixing; (3) adding to the mixture at a stage in the process of mixing 75 the charcoal and energizer and pulverizing the latter, coal tar in a quantity to render the mixture coherent and moldable; (4) molding said coherent mixture into briquettes; (5) shrinking such briquettes by 80 baking them to dryness at a temperature less than adequate to fuse the energizer; (6) crushing the briquettes and screening and sorting the crushed material to sizes.

2. A carburizing material consisting of 85 dried and shrunken briquettes composed of charcoal and an energizer with a binder.

In testimony whereof, I have hereunto set my hand at Chicago, Illinois, this 9th day of February, 1921.

LOUIS AEBY.